# EUROPEAN PATENT SPECIFICATION

(11) **EP 0 130 065 B1**
(45) Date of publication and mention of the grant of the patent: **23.11.1988**
(21) Application number: 84304239.1
(22) Date of filing: 22.06.1984
(51) Int. Cl.: C10L 10/00

(54) **Improvements in and relating to combustion**
Verbesserung in bezug auf die Verbrennung
Amélioration concernant la combustion

(30) Priority: 22.06.1983 GB 8316937
(43) Date of publication of application: 02.01.1985
(73) Proprietor: Hardy, Leonard Rhys, Desford Leicester LE9 9JJ (GB); Ayre, Richard Geoffrey, Thurcaston Leicester (GB)
(72) Inventor: Hardy, Leonard Rhys, Desford Leicester LE9 9JJ (GB); Ayre, Richard Geoffrey, Thurcaston Leicester (GB)
(74) Representative: Hallam, Arnold Vincent

(56) References cited:
- DE-A- 2 361 091
- FR-A- 2 510 237
- GB-A- 1 335 462
- US-A- 4 191 115
- Second interim report on external deposits and corrosion in boiler plant (1946-1951), The Boiler Availibility Committee, London, 1953 pages 3-7, 21
- Journal of the Institute of Fuel, February 1968 pages 63-65, "The formation of alkali-rich deposits by a high chlorine coal".

## Description

The present invention relates to the reduction of undesirable combustion by-products in boilers, incinerators and similar plant.

A major problem associated with the combustion of fossil fuels in, for example, boilers is the considerable amount of adherent scale, soot and smut deposits which build up in the boiler combustion chambers, flue systems and chimneys. The effect of these deposits in the boiler tubes is to reduce boiler heat transfer rates dramatically, resulting in considerable increases in fuel consumption. Regular cleaning by vigorous mechanical means to remove these deposits is therefore necessary to maintain a reasonable level of boiler efficiency, which causes damage to the tubes and is both time consuming and expensive. Also, this often requires the use of a "back-up" boiler while the main boiler is shut down for cleaning. Additionally, smut deposits within the flue passes become entrained in the flue gases during load fluctuations causing smut emission and deposition in the immediate locality.

The above-mentioned problems are well known in the art and many attempts have been made to overcome them. For example, organic compounds containing metals such as lead, cobalt, manganese, copper, nickel and chromium chromium can under certain conditions function as soot destroyers or combustion aids and it has been proposed to add these metals to fuels to provide for more complete combustion of the fuel to C0₂ and H₂0. However, the relatively large amounts of these metals which must be added to the fuel to give a significant improvement causes the fuel to become so unstable that the catalytic properties of these metals cannot be used. This effect can be offset by adding stabilisers or antioxidants to the fuel but again, large amounts are required which renders this economically impractical and gives rise to further disadvantageous secondary effects.

It has also been proposed to add lead or cobalt soaps to fuel to reduce soot but again considerable problems are caused by the resulting unwanted byproducts.

It has also been suggested that a mixture of compounds of manganese or copper and lead, cobalt, nickel, zinc, chromium, antimony, tin or vanadium in specified proportions can prove effective, in improving the burning properties of fuel without serious side effects and that the improvement is not obtained when using a compound of only one of the metals.

DE-A-2 361 091 and FR-A-2 510 237 describe the feeding of additives including oxides of various metals into a combustion chamber in order to remove gaseous harmful substances such as sulphur, chlorine and flourine compounds.

Accordingly, the present invention provides a combustion process comprising passing combustion air over an ignited fossil fuel in a combustion chamber and prior to or during combustion introducing in the combustion chamber a measured quantity of finely divided ferric oxide such that the amount of solid combustion by-products deposited in flue passes and chimneys of the combustion chamber during the combustion process is reduced, and wherein said measured quantity is in the range 0.1134 Kg to 0.4536 Kg for an amount of fossil fuel being the thermal equivalent of 1 tonne of coal.

Preferably the substance is introduced during the combustion process, although it may also be introduced prior to combustion in the fuel.

The present invention stems from the unexpected discovery that the addition into the combustion zone of finely divided ferric oxide particles alone or mixed with an inert material in small quantities significantly reduces the formation and deposition of scale, smut and other solid combustion by-products and also acts to reduce existing scale. This results in the maintenance of heat transfer rates for very much longer periods and improved plant performance than in the absence of the substance with consequent saving in fuel consumption and maintenance costs.

Finely divided iron oxide is introduced into the combustion chamber in the form of ferric oxide (Fe₂0₃). The substance is preferably blown into or over the combustion zone repeatedly over short periods of time at intervals as desired, as a fine powder during combustion either in the combustion air or separately. The quantity of ferric oxide required to achieve the desired effect is very small, depending on the quality and type of the fuel. The substance may alternatively or additionally be added to the fuel itself and although the substance is described as being added during combustion it will be appreciated that quantities can be added prior to combustion. The substance may also be added continuously if desired and can be in the form of a powder, a suspension in a substantially inactive or combustible liquid, or in the form of small pellets.

Dosage rate of the substance is 0.1134 Kg (0.25 lbs) to 0.4536 Kg (1 Ib) per tonne of coal consumed, or the thermal equivalent of oil, gas and other fossil fuels.

The quantities of substance injected into the combustion chamber, because they are so small, can be more easily controlled by first mixing the substance intimately with a neutral powder. This also aids dispersion of the substance throughout the chamber. A diluent powder composed, for example, of bentonite, synthetically organically modified bentonite, dolomite or calcined dolomite or other finely divided diluent powder which is inactive i.e. does not adversely affect the process of the present invention may be used.

In the combustion chamber itself, during combustion the ferric oxide causes an alteration in the character of existing scale deposits within the chamber, flue passes and chimney, the deposits becoming friable and easily removed. The property of the scale which causes it to adhere strongly to the boiler heat transfer surfaces, ducts and chimneys is reduced as a result of which the scale becomes detached from these areas and falls away, allowing for a greater rate of heat transfer and therefore increased boiler efficiency and performance. In addition, since this avoids the need for abrasive cleaning methods the life of the boiler tubes is improved. Further scale formation is reduced and the soot and carbonaceous content of deposits in the tubes and flues is reduced enabling easier removal. Smut content is also reduced in the boiler flue deposits resulting in a generally free-flowing powder which is easily removed and contains fewer oil and other carbon compounds. Acid smut emission due to entrainment of smut in the flue gases is considerably reduced.

The overall effect, therefore, is a cleaner combustion chamber, flue passes and chimneys resulting in the maintanence of the boiler at higher efficiency and performance for long periods with consequently lowered fuel costs, a significant reduction in the cost of maintenance and cleaning and reduction in smut emission due to entrainment.

The ferric oxide may conveniently be mixed with a combustible liquid to inhibit coagulation.

The following examples are typical of the results achieved by the process of the present invention in some 30 installations involving Thompson (Registered Trade Mark) Cochran, Danks, Hartley & Sugden, Centrax (Registered Trade Mark) Robey, Vekos and Trianco (Registered Trade Mark) boilers of various capacities for industrial and domestic use.

### Example 1

A mixture of iron oxide (Fe₂0₃) as 30% by weight in an inactive finely divided naturally occurring clay powder was injected into the combustion chamber of a Colifax Hot Water boiler in the proportion of 0.227 Kg (0.5 lbs) weight of the mixture to each tonne of coal consumed. The powder was injected every 3 hours for the requisite period to achieve the above dose rate.

The boiler had not been cleaned prior to the use of the powder and contained adherent scale.

The boiler efficiency as measured by flue gas analysis and temperature method improved from 65% to 71 % over a period of 6 days and was associated with the removal of substantially all the adherent scale.

The reduction in the carbonacous content of the boiler flue passes was some 50% as measured in before and after conditions.

### Example 2

A mixture of iron oxide (Fe₂0₃) as 25% by weight in an inactive powder was injected as for Example 1 into the combustion chambers of three Centrax coal-fired boilers over a period of 6 months. The boilers became free from adherent scale within the first 3 to 4 weeks and the flue deposits become substantially free from soot and greasy smut which made them extremely free flowing and easily removed.

Heavy falls of hard sooty scale occurred in the breach ducts and stack which, once removed, left the passes in an almost new condition.

Fuel savings of 11% overall were recorded after allowing for seasonal differences in ambient conditions.

### Example 3

Iron oxide (Fe₂0₃) was injected or added to the coal in a number of smaller coal-fired domestic boilers over a period of some 6 months. All boilers, although initially heavily contaminated with scale and soot deposits soon became substantially free of deposits with very little cleaning being necessary (and then only with a brush) once the main detached scale debris was removed.

### Example 4

A 40% mixture by weight of iron oxide (Fe₂0₃) mixed with a neutral clay based powder was injected into the combustion chamber of a Ther- max oil fired (3500 secs.) boiler at the rate of 0.1134 Kg (0.25 lbs.) per 300 galls. of oil consumed. Although new, prior to the injection of the iron oxide mix the boiler was subject to heavy deposition of hard scale on the flue side of the boiler tubes which was difficult to remove and meant that the boiler had to be shut down monthly for cleaning.

The injection of the iron oxide mixture removed the hard scale and prevented further formations. As a result the boiler was operated for a period of 4 months without any deterioration in performance or shut down for cleaning being necessary.

An accurate evaluation of the fuel savings achieved by the use of iron oxide (Fe₂0₃) is difficult to establish because of the many variables involved and the well known difficulties encountered in monitoring boiler performance accurately even with the most sophisticated instrumentation. It will be appreciated, however, that it is self evident that a boiler which is free from adherent scale, soot and smutty products will give a substantially better performance than one which is not free of such deposits and the boiler condition will be obvious on inspection and sophisticated instrumentation would not be required to establish this.

## Claims

1. A combustion process comprising passing combustion air over an ignited fossil fuel in a combustion chamber and prior to or during combustion introducing in the combustion chamber a measured quantity of finely divided ferric oxide such that the amount of solid combustion by- products deposited in flue passes and chimneys of the combustion chamber during the combustion process is reduced; and wherein said measured quantity is in the range 0.1134 Kg to 0.4536 Kg for an amount of fossil fuel being the thermal equivalent of 1 tonne of coal.

2. A combustion process as claimed in claim 1 wherein said ferric oxide is introduced during the combustion process.

3. A combustion process as claimed in claim 1 or 2 wherein said ferric oxide is introduced into the combustion chamber as a powder.

4. A combustion process as claimed in any of claims 1 to 3 wherein prior to the introduction of said ferric oxide into the combustion chamber the ferric oxide is mixed substantially uniformly with a substantially inert material.

5. A combustion process as claimed in claim 4 wherein said ferric oxide is a finely divided powder and is uniformly mixed with a diluent powder selected from at least one of the following: bentonite, synthetically organically modified bentonite, dolomite, calcined dolomite.

6. A combustion process as claimed in any of claims 1 to 5 wherein said ferric oxide is mixed with a combustible liquid to inhibit coagulation.

7. A combustion process as claimed in any of claims 1 to 6 wherein said ferric oxide is introduced into the combustion chamber over the fuel combustion area.

8. A combustion process as claimed in any of claims 1 to 8 wherein said ferric oxide is introduced into the combustion chamber at discrete intervals of time.

## Patentansprüche

1. Verbrennungsprozeß, bei dem in einer Brennkammer Verbrennungsluft über einen entzündenten fossilen Brennstoff geleitet wird, bei dem vor oder während der Verbrennung in die Brennkammer eine richtig bemessene Menge an feinverteiltem Eisenoxid derart eingeleitet wird, daß die Menge an festen Verbrennungsprodukten, welche in den Rauchzügen und Rauchfängen der Brennkammer während des Verbrennungsprozesses abgelagert werden, reduziert wird, und wobei die richtig bemessene Menge im Bereich von 0,1134 kg bis 0,4536 kg pro der einer Tonne Kohle thermisch äquivalenten Menge von fossilem Brennstoff liegt.

2. Verbrennungsprozeß nach Anspruch 1, dadurch gekennzeichnet, daß das Eisenoxid während des Verbrennungsprozesses eingeleitet wird.

3. Verbrennungsprozeß nach Anspruch 1 oder 2, dadurch gekennzeichnet, daß das Eisenoxid in die Brennkammer als Pulver eingeleitet wird.

4. Verbrennungsprozeß nach mindestens einem der Ansprüche 1 bis 3, dadurch gekennzeichnet, daß vor dem Einleiten des Eisenoxids in die Brennkammer dieses weitgehend gleichmäßig mit einem im wesentlichen inerten Material vermischt wird.

5. Verbrennungsprozeß nach Anspruch 4, dadurch gekennzeichnet, daß das Eisenoxid feinverteiltes Pulver ist und mit einem pulverförmigen Streckmittel gleichmäßig vermischt wird, das aus wenigstens einen der folgenden Stoffe ausgewählt wird: Bentonit, synthetisch, organisch veränderter Bentonit, Dolomit, gebrannter Dolomit.

6. Verbrennungsprozeß nach mindestens einem der Ansprüche 1 bis 5, dadurch gekennzeichnet, daß das Eisenoxid mit einer brennbaren Flüssigkeit vermischt wird, um ein Zusammenbacken zu verhindern.

7. Verbrennungsprozeß nach mindestens einem der Ansprüche 1 bis 6, dadurch gekennzeichnet, daß das Eisenoxid in die Brennkammer über die Brennstoff-Verbrennungszone eingeleitet wird.

8. Verbrennungsprozeß nach mindestens einem der Ansprüche 1 bis 7, dadurch gekennzeichnet, daß das Eisenoxid in die Brennkammer in diskreten Zeitabständen eingeleitet wird.

## Revendications

1. Procédé de combustion qui comprend le passage de l'air de combustion sur un combustible fossile en ignition dans une chambre de combustion et, avant ou pendant la combustion, l'introduction, dans la chambre de combustion, d'une quantité mesurée d'oxyde ferrique finement divisé telle que la quantité de sous-produits de combustion solides déposés dans les carneaux et cheminées de la chambre de combustion pendant le procédé de combustion soit réduite, et dans lequel cette quantité mesurée se situe dans l'intervalle de 0,1134 kg à 0,4536 kg pour une quantité de combustible fossile qui est l'équivalent thermique de 1 tonne de charbon.

2. Procédé suivant la revendication 1, dans lequel l'oxyde ferrique est introduit pendant le procédé de combustion.

3. Procédé de combustion suivant la revendication 1 ou 2, dans lequel l'oxyde ferrique est introduit à l'état de poudre dans la chambre de combustion.

4. Procédé de combustion suivant l'une quelconque des revendications 1 à 3, dans lequel, avant l'introduction de l'oxyde ferrique dans la chambre de combustion, l'oxyde ferrique est mélangé en substance uniformément avec une matière sensiblement inerte.

5. Procédé de combustion suivant la revendication 4, dans lequel l'oxyde ferrique est une poudre finement divisée et est mélangé uniformément avec une poudre de dilution choisie parmi au moins l'un des agents suivants: betonite, bentonite modifiée synthétiquement par un agent organique, dolomie et dolomie calcinée.

6. Procédé de combustion suivant l'une quelconque des revendications 1 à 5, dans lequel l'oxyde ferrique est mélangé avec un liquide combustible pour inhiber la coagulation.

7. Procédé de combustion suivant l'une quelconque des revendications 1 à 6, dans lequel l'oxyde ferrique est introduit dans la chambre de combustion sur la zone de combustion du combustible.

8. Procédé de combustion suivant l'une quelconque des revendications 1 à 7, dans lequel l'oxyde ferrique est introduit dans la chambre de combustion à intervalles distincts dans le temps.
